

# UNITED STATES PATENT OFFICE.

GILBERT RIGG, OF PALMERTON, PENNSYLVANIA, ASSIGNOR TO NEW JERSEY ZINC COMPANY, OF NEW YORK, N. Y., A CORPORATION OF NEW JERSEY.

## PROCESS OF PREPARING PYRITIFEROUS ZINC-BLENDE FOR MAGNETIC SEPARATION.

1,103,082.

Specification of Letters Patent.

Patented July 14, 1914.

No Drawing.

Application filed March 27, 1911. Serial No. 617,211.

*To all whom it may concern:*

Be it known that I, GILBERT Rigg, a subject of the King of Great Britain, residing at Palmerton, county of Carbon, State of Pennsylvania, have invented certain new and useful Improvements in Processes of Preparing Pyritiferous Zinc-Blende for Magnetic Separation; and I do hereby declare the following to be a full, clear, and 10 exact description of the invention, such as will enable others skilled in the art to which it appertains to make and use the same.

This invention relates to a process for separating pyrite from zinc blende and other 15 minerals with which it is associated, by first converting the pyrite into pyrrhotite or magnetic sulfid, with the simultaneous recovery of the sulfur in elementary form, and thereupon withdrawing the pyrrhotite from the 20 zinc blende or other non-magnetic material by means of magnetic attraction.

In the usual method of converting pyrite ( $FeS_2$ ), into pyrrhotite, the ore is partially roasted in a current of air, and the endeavor 25 is made to interrupt the roasting at a point when sufficient sulfur has been driven off to effect the desired conversion into pyrrhotite, whose formula varies somewhat but is usually given as from  $Fe_7S_8$  to  $Fe_{11}S_{12}$ . If 30 the roasting is not continued long enough, a certain amount of non-magnetic pyrite is left unchanged, and if carried too far, non-magnetic ferric oxide is produced, which is equally undesirable from the standpoint of 35 effecting its subsequent separation. Moreover, there is a further objection to converting the pyrite of the ore into pyrrhotite by partially roasting in a current of air, in that the sulfur is driven off as  $SO_2$  mixed with 40 large volumes of fire gases, so that the gas mixture is too dilute and too impure to be available for sulfuric acid manufacture. The gas mixture is, therefore, usually delivered into the air, and not only is the sulfur 45 wasted, but the gases thus discharged are very injurious to vegetation and cause much trouble.

By the practice of my invention, as hereinafter described, it is impossible to pass 50 beyond the point of converting the pyrite into pyrrhotite or magnetic sulfid, and the sulfur is recovered in the form of elementary sulfur or brimstone, all loss and nuisance being practically obviated.

In carrying the process into effect, I heat 55 the pyritiferous ore in a muffle, or in a shaft, from which the fire gases and air are excluded. At temperatures ranging from 600° C. to 800° C. the pyrite gives up part of its sulfur, which passes over as sulfur vapor, 60 and, leaving the muffle or shaft by suitable exit openings, is recovered in the form of elementary sulfur in a suitable condenser. The pyrite by this treatment, is converted 65 into pyrrhotite or magnetic sulfid and may thereupon be separated from the zinc blende or other non-magnetic minerals with which it is associated, by means of a magnetic separator. As hereinbefore noted, it is a characteristic feature of this method of treatment 70 that it is impossible to pass beyond the point of converting the pyrite into pyrrhotite or magnetic sulfid. After it has been so converted, further heating has no effect upon it, unless the temperature is carried 75 to such a degree as to fuse the charge, and this is easily avoided. Consequently, the heating can be continued long enough to insure the complete conversion of the pyrite into pyrrhotite without incurring any 80 danger from over-roasting. This insures the ultimate withdrawal by the magnetic separator from the zinc blende or other non-magnetic constituent of the ore of practically all of the pyrite originally contained 85 therein, with the incidental recovery of the elementary sulfur as a valuable by-product and the avoidance of injury to vegetation which would be involved in discharging the sulfur in the form of  $SO_2$  into the atmosphere. 90

Having thus described my invention, what I claim is:

1. The process of treating zinc blende associated with pyrite, so as to render said constituents capable of magnetic separation, which consists in expelling a portion of the sulfur of the pyrite by heating the pyritiferous ore at a temperature below the fusing point of the pyrite and below the dissociation point of the zinc blende, thereby 95 converting the pyrite constituent of the ore into a magnetic condition as pyrrhotite, and without altering the zinc blende constituent; substantially as described. 100

2. The process of treating zinc blende associated with pyrite, so as to render said constituents capable of magnetic separation,

which consists in heating the pyritiferous ore, with the exclusion of air, thereby expelling a portion of the sulfur of the pyrite constituent of the ore and converting it into a magnetic condition as pyrrhotite, the heating operation being conducted at a temperature below the fusing point of the pyrite, whereby said conditions of the operation insure against such desulfurization as would

carry the pyrite beyond the magnetic condition; substantially as described.

In testimony whereof I affix my signature, in presence of two witnesses.

GILBERT RIGG.

Witnesses:

HENRY HARDENBERGH,  
E. G. TACY.